

1

2,840,498

## COMPOSITION AND METHOD FOR PRODUCING COMBINATION CORROSION RESISTANT AND LUBRICATING COATINGS ON METALS

Earl Eugene Logue, Jr., Birmingham, and Ernest P. Bell, Detroit, Mich., assignors to Parker Rust Proof Company, Detroit, Mich., a corporation of Michigan

No Drawing. Application June 8, 1953  
Serial No. 360,353

10 Claims. (Cl. 148—6.15)

This invention relates to a composition and method for producing a coating on metallic surfaces and particularly ferrous surfaces which functions both as a corrosion-resistant coating and as a lubricant in operations which deform the metal, such as drawing.

In the cold working of metals, it is customary to employ a lubricant to aid in reducing the friction between the moving metal surfaces, which friction in the absence of a lubricant actually causes a tearing of the metal and/or galling of the dies being used. Ordinary lubricating oils or extreme pressure lubricating oils have been successfully used in the drawing of some of the softer metals, but these materials have not been successful in the deforming of the harder metals, especially where the deformation is relatively severe. The harder metals such as iron, steel, stainless steel and the extremely hard alloy steels have been successfully deformed by preliminarily coating the metal surface with an underlayer of a protective chemical coating such as a phosphate, oxide, sulfide or oxalate together with an overlayer of a conventional lubricant. Such conventional lubricants have included ordinary lubricating oils; extreme pressure lubricating oils; fats or soaps in aqueous and dry form; and fats, oils, or soaps in combination with a variety of infusible pigments such as clay, graphite, mica, etc. In employing the combination of a chemical coating and a lubricant, it has been necessary heretofore to employ separate compositions and sequential steps of first treating the metal with a phosphate solution, then a first rinse in water and a second rinse in water or a slightly alkaline solution, and thereafter treating the phosphate coated article in a suitable lubricant composition.

It is the principal object of this invention to provide a single composition which produces on a metallic surface a coating which is both protective and has lubricating properties enabling relatively severe deformation of harder metals such as iron and steel.

Another object is to provide a method for forming on a metallic surface an integral chemical coating which has lubricating properties.

A further object is to provide an inexpensive composition and a simple one-step method, which eliminates the necessity for using the customary two-stage rinsing, for producing an integral chemical coating having lubricating properties on metallic surfaces, and particularly ferrous surfaces. A still further object is to provide an aliphatic phosphate coating on metal surfaces which has lubricating properties. Other objects and advantages of the invention will appear in the following detailed description of the invention.

These and related objects are accomplished in accordance with this invention by coating the surfaces of metals, particularly ferrous metals, by contacting the surface with an aqueous dispersion or admixture containing as the essential coating producing ingredients an aliphatic ester of phosphoric acid having from 8-18 carbon atoms, and a metallic ion that forms a salt with the aliphatic ester of phosphoric acid which is compatible with the disper-

2

sion, said dispersion or admixture having a controlled acidity within a range of pH of about 3.0 and 5.5. By "compatible with the dispersion" is meant that the metallic salt of the aliphatic phosphate is soluble in or at least semi-soluble or readily dispersible in the aqueous solution or dispersion of the aliphatic ester. The coating which is formed by this treatment has a velvety appearance and is an amorphous type of coating, being partially greasy and capable of being crushed to a continuous unctuous film so that it is well suited for use as a lubricant in metal deformation operations. The coating is exceptionally adherent and resists removal from the surface of the metal even when the highest pressures normally encountered in deformation operations are used. In addition to the aliphatic phosphoric acid ester and the metallic salt thereof, the composition may also contain an amine which is reactive with a portion of the aliphatic phosphoric acid ester to form a compatible amine salt thereof and an oxidizing or accelerating agent which is conventionally employed in phosphate solutions of the coating-phosphate type such as zinc or manganese phosphates.

The degree of acidity of the compositions of this invention has been found to be critical and it is to be understood that the incorporation of an amine which forms a compatible amine salt with the aliphatic phosphoric ester is but one means of achieving the desired degree of acidity and that the benefits of the invention may be obtained in the absence of either or both the amine and the accelerating agent. It is to be further understood, however, that the incorporation of an amine in the basic composition produces a preferred composition for reasons which will be explained in greater detail hereinafter, and that the best solutions of this invention also include an accelerating agent or agents.

The aliphatic esters of phosphoric acid which, in combination with a metallic salt of such ester, have been found to be useful for the purposes of this invention, are the esters which may be regarded as the reaction products of phosphoric acid with aliphatic alcohols containing from 8-18 carbon atoms. The aliphatic portion of the ester may be either saturated or unsaturated. While the saturated alcohols are somewhat more readily commercially available, the unsaturated aliphatic esters having unsaturation of the olefinic type have nevertheless been found to be equally suitable in the compositions of this invention. When the length of the carbon chain in the ester is less than 8 carbon atoms, the coating which is produced does not exhibit the characteristics of a lubricant to a desirable degree, and when the length of the carbon chain exceeds about 18 carbon atoms, the aliphatic phosphate ester is insufficiently dispersible in water to form a workable material. Preferred materials for the purposes of this invention are the lauryl esters and the oleyl esters. Mixtures of esters having carbon chain lengths between 8 and 18 may be used, and mixtures of esters actually represent a preferred form of the invention because alcohols of mixed carbon chain length are readily available and the mixed esters are easily obtained. Proportions of esters which have been found to be suitable are in the range of about 3 grams/liter to about 20 grams/liter of the monolauryl phosphoric acid ester which is sometimes designated monolauryl acid phosphate. Equivalent proportions of other monoesters having 8 to 18 carbon atoms may be satisfactorily used.

Any of a wide variety of metallic ions may be used in the compositions of this invention. The only apparent restriction upon the type of metallic ion which is suitable, is that the metallic ion must be capable of forming with the aliphatic phosphoric acid ester, a salt which is soluble, or at least semi-soluble or readily dispersible in the aqueous dispersion of the aliphatic phosphoric acid ester.

Typical metallic ions which have been found to be useful for this purpose include zinc, aluminum, the alkali metals including ammonium, cadmium, copper, nickel and iron. While it is possible to obtain a greasy film from an aqueous dispersion containing only an aliphatic phosphoric acid ester having 8-18 carbon atoms, the film so produced is of inferior quality, has poor adhesion and appears to be an adsorbed film rather than an integral chemical coating. The presence of a compatible metallic ion in the compositions of this invention apparently imparts to the aqueous dispersion of aliphatic phosphoric acid ester, the ability to chemically react with the surface and to form a velvety coating of amorphous nature, which coating is integrally bonded to the metal surface. The coating resulting from compositions containing both an aliphatic phosphoric acid ester having 8-18 carbon atoms and a compatible metal ion are sufficiently adherent and possessed of a greasy nature such that upon the application of pressure, the velvety, amorphous coating is crushed into a continuous film having good lubricating properties and high resistance to being dislodged due to the application of pressure.

The proportion of metallic ion which is necessary for the formation of the superior coatings of this invention is relatively restricted. In the operating solutions, the metallic ion content may satisfactorily vary between about 0.3 gram per liter and 11.0 grams per liter of zinc or the equivalent proportion of other suitable metallic ion, such as those enumerated hereinabove. When the metallic ion content drops below the equivalent of 0.3 gram/liter of zinc, the coating is a relatively non-adherent greasy film, whereas when the concentration of metallic ion exceeds the equivalent of 11 grams per liter of zinc, the salt of the ester cannot be maintained in dispersion and precipitation occurs.

The metallic ion is preferably introduced into the composition as a salt and only limited quantities may be introduced as basic salts or hydroxides. When a relatively high concentration of metallic ion is desired, introduction of the metallic ion as a basic salt or a hydroxide is not feasible since the pH is raised above the operable limit before the desired concentration is achieved. In this case, metallic salts such as the acetates or nitrates should be employed, and the pH adjusted with the amine being employed. The use of salts containing a halide, such as chloride, bromide or iodide is not recommended.

The incorporation of an amine in the basic composition of this invention tends to increase the solubility of the metallic salt of the aliphatic phosphate in the dispersion. For the purpose of obtaining coatings which are relatively heavy and which are especially suited for sever deformation operations, it is desirable to maintain the concentration of the metallic salt near the maximum degree of its solubility. The presence of an amine additionally raises the pH of the solution and provides a convenient means of both achieving maximum solubility of metallic salt in the dispersion and regulating the pH within the desired range of 3.0 to 5.5. Amines which are suitable for this purpose include those amines which upon reaction with the aliphatic phosphoric acid ester having from 8-18 carbon atoms produce a soluble salt of the ester and impart the above referred to effects. Ammonia, monoamines, diamines, tertiary amines, cyclic and heterocyclic amines are useful for this purpose. Typical specific representatives of the amines which have been found to be suitable are ethanol amine, isopropyl amine, hydrazine, 3-isopropoxy-propylamine, triethanol amine and morpholine. The proportion of amine which may be used is that amount which produces the desired pH within the range of 3.0-5.5.

The numerical pH limits of 3.0 to 5.5 refer to a pH determined with Hydron papers. It has been found that although the absolute degree of precision generally obtainable with Hydron papers is less than that of glass electrodes, the reproducibility and accuracy of the pH

determinations with Hydron papers for the dispersions of this invention are actually better than those obtainable using glass electrodes.

The compositions of this invention from the desired coatings in a shorter period of time when they include an accelerating or oxidizing agent. Any oxidizing agent which is conventionally employed for the purpose of accelerating the formation of a coating from a solution such as zinc phosphate or manganese phosphate solution, may be used for the purposes of this invention. Typically useful oxidizing agents include the nitrites, nitrates, peroxides, chlorates, bromates, sulfites and nitro-organic compounds such as m-nitrobenzene sulfonate and picric acid. For convenience, the oxidizing agents may be added as the metallic salts such as the sodium or other alkali metal salt, and the proportion of metallic ion so introduced is small and relatively insignificant to the overall metallic ion content. Suitable concentrations of these oxidizing agents which may be employed to decrease the time required for producing the coatings of this invention are 0.3%-0.5% sodium meta-nitro benzene sulfonate; 0.01%-0.5% picric acid; 0.05-0.3% hydrogen peroxide; 0.03%-5.0% chlorate; 0.03%-0.5% bromate; 0.01%-0.15% nitrite; 0.02%-0.15% sulfite; 0.03%-2.0% nitrate; 0.01%-0.3% hydroxylamine.

Broadly stated, the method of this invention comprises the steps of contacting the metal surface to be treated with the compositions of this invention and thereafter drying the coating thus formed on the metallic surface. As is usual with phosphate coating solutions, it is desirable to apply the compositions of this invention while hot and to regulate the time of solution contact with the metal surface and the concentration of the solution so as to produce the desired thickness of coating. Temperatures between about 90° F. and 190° F. may be employed. The step of drying the coating on the metal surface is preferably performed at an elevated temperature less than about 250° F., though where the time required for fully preparing the metal surface to be drawn is unimportant, the coating may be dried in air. Where the coating is dried by subjecting the same to an elevated temperature, a somewhat increased degree of reaction with the metal surface is thought to occur and the resultant coating is somewhat improved in its adherence to the metal surface. Drying the coating at an elevated temperature represents the preferred procedure.

The examples given below illustrate in greater detail typical compositions of, and the method of this invention.

#### EXAMPLE I

A mixture was prepared by heating together 26.5 grams of monolauryl phosphoric acid and 4 grams of zinc oxide with 500 ml. of water and mixing in a Waring blender. The resultant mixture had a pH of 1.2 which was adjusted with sodium carbonate to 5.5. Clean, mild steel panels were immersed in the solution at 170° F.-180° F. for periods of one-half minute to two minutes, withdrawn and dried. All the panels were coated with a smooth, adherent, water repellent coating which was somewhat dusty in appearance. The coatings crushed to a thin unctuous film on the application of pressure.

#### EXAMPLE II

|                                   | Grams |
|-----------------------------------|-------|
| Monolauryl phosphate              | 160   |
| Morpholine                        | 32    |
| Zinc acetate                      | 25    |
| Sodium chlorate                   | 35    |
| Distilled water to make 2 gallons |       |

The emulsion containing the above ingredients was stable and had a pH of 5.0. Three hundred and fifteen 4" x 6" steel panels were processed through the solution at 140° F.-150° F. for 5 minutes each. Smooth adherent coatings were formed which were slightly more unctuous than the coatings of Example I.

A number of formulations were prepared corresponding to that set forth above in Example II except the morpholine was omitted, and in separate formulations was replaced by a chemically equivalent proportion of ammonia, triethanolamine, hydrazine, and 3-isopropoxypropylamine. Steel panels treated in these modified solutions in the same manner were coated with coatings generally similar to those obtained when morpholine was present.

## EXAMPLE III

A 100 gallon aqueous emulsion was prepared containing:

|                                            | Pounds |
|--------------------------------------------|--------|
| Monolauryl phosphoric acid                 | 15.5   |
| Morpholine                                 | 3.2    |
| Zinc acetate $Zn(C_2H_5O_2)_2 \cdot 2H_2O$ | 3.4    |
| Sodium chloride                            | 3.4    |

The pH of the solution was adjusted upwardly to 5.3 by adding 1 liter of concentrated ammonium hydroxide. A number of pieces of steel tubing were immersed in the solution at 140° F.-150° F. for 5 minutes, withdrawn and force dried. The coatings were uniformly smooth and adherent.

Several pieces of  $\frac{1}{2}$  inch outside diameter steel tubing having a wall thickness of 0.015" were so coated and drawn to 0.400" outside diameter x 0.014" wall thickness, and immediately redrawn to 0.345" outside diameter x 0.0115" wall thickness for a total reduction of 47%. The temperature of the tubing during drawing remained low and the surface of the drawn tubing was good.

The chemicals in the emulsion are depleted as the emulsion is used for coating, and may be easily replenished by the use of a replenishing concentrate. Suitable formulations for replenishing or for original make-up are given below:

## Formula I

|                                  |        |     |
|----------------------------------|--------|-----|
| Lauryl acid phosphate            | grams  | 600 |
| Oleyl acid phosphate             | do     | 750 |
| Stearyl acid phosphate           | do     | 790 |
| Morpholine                       | do     | 150 |
| Sodium hydroxide                 | do     | 75  |
| Sodium acetate.3H <sub>2</sub> O | do     | 188 |
| Ferric nitrate.9H <sub>2</sub> O | do     | 188 |
| Distilled water                  | liters | 4   |

This concentrate is in the form of a heavy paste and is best compounded by heating the acids to melting and adding the morpholine thereto at about 200° F. and maintaining the temperature until the reaction is complete. The sodium hydroxide may be dissolved in part of the water and the acetate and nitrate in the balance and both solutions heated to about 150° F. While the caustic is being stirred, the mixture of acids with morpholine and the acetate-nitrate solution are added slowly and after about 15 minutes of mixing a uniformly blended heavy paste is obtained. A working solution may be prepared by using about 60 to 70 pounds of this concentrate per 100 gallons of solution or emulsion, and adding an oxidizing agent thereto.

## Formula II

|                                  | Grams |
|----------------------------------|-------|
| Monolauryl acid phosphate        | 15    |
| Mono-oleyl acid phosphate        | 7     |
| Morpholine                       | 7     |
| Ferric nitrate.9H <sub>2</sub> O | 6     |
| NaOH                             | 1     |

Distilled water to make 250 ml.

This formulation when mixed as described above in 70 Formula I, produced a heavy, creamy material.

What is claimed is:

1. A composition of matter comprising an aqueous dispersion consisting essentially of water, a mono-aliphatic phosphoric acid ester having from 8 to 18 carbon atoms,

5 a metal ion which forms a salt with the said phosphate and which is compatible with said dispersion in an amount equivalent to about 0.3-11 grams/liter of zinc, and an amine in an amount sufficient to produce a pH between about 3.0 and 5.5.

2. A composition of matter comprising an aqueous dispersion consisting essentially of water, a mono-aliphatic phosphate having from 8 to 18 carbon atoms, a metallic ion in an amount equivalent to about 0.3-11 grams/liter 10 of zinc, an oxidizing agent and an amine in an amount sufficient to produce a pH between about 3.0 and 5.5.

3. A composition of matter comprising an aqueous dispersion consisting essentially of water, a monoaliphatic phosphate having from 8 to 18 carbon atoms in an 15 amount from about 3 to 80 grams per liter, a metallic ion which yields with said phosphate a salt which is at least semi-soluble in said dispersion and which is present in an amount equivalent to about 0.3 to 11 grams per liter of zinc, an oxidizing agent, and an amine in an 20 amount sufficient to produce a pH of between about 3.0 and 5.5.

4. The method of forming on a metallic surface an integrally bonded chemical coating having lubricating properties which comprises the steps of contacting the 25 metal surface with an aqueous dispersion consisting essentially of water, an aliphatic phosphate having 8 to 18 carbon atoms and a metal ion which yields a salt which is at least semi-soluble in said dispersion in an amount equivalent to about 0.3-11 grams/liter of zinc 30 and having a pH of about 3.0 to 5.5, and thereafter drying the said coating at an elevated temperature.

5. The method of forming on the surface of a ferrous article an integrally bonded chemical coating having lubricating properties which comprises the steps of immersing the article in an aqueous dispersion at a temperature between about 90° F. and 190° F. for a short time, which dispersion consists essentially of water, a monoaliphatic phosphate having 8 to 18 carbon atoms in an amount of about 3 to 80 grams per liter and a metallic ion which yields with said phosphate a salt which is at least semi-soluble in said dispersion in an amount equivalent to about 0.3 to 11 grams per liter of zinc, said dispersion having a pH between about 3 and 5.5, and thereafter drying said coating at an elevated temperature less than about 250° F.

6. The method of forming on the surface of a ferrous article an integrally bonded chemical coating having lubricating properties which comprises the steps of immersing the article in an aqueous dispersion at a temperature between about 90° F. and 190° F. for a short time, said dispersion consisting essentially of water, a monoaliphatic phosphate having from 8-18 carbon atoms and a metallic ion which yields with said phosphate a salt which is at least semi-soluble in said dispersion in an amount equivalent to about 0.3-11 grams/liter of zinc, an oxidizing agent and an amine, said dispersion having a pH between about 3.0 and 5.5, withdrawing the article, and drying the coating thereon.

7. The method of forming on the surface of a ferrous article an integrally bonded chemical coating having lubricating properties which comprises the steps of immersing the article in an aqueous dispersion at a temperature between about 90° F. and 190° F. for a short time, said dispersion consisting essentially of water, a mono-aliphatic phosphate having from 8 to 18 carbon atoms in an amount from about 3 to 80 grams per liter, a metallic ion which yields with said phosphate a salt which is at least semi-soluble in said dispersion and which is present in an amount equivalent to about 0.3 to 11 grams/liter of zinc, an oxidizing agent, and an amine in an amount sufficient to produce a pH of between about 3.0 and 5.5.

8. A metallic surface having thereon a metallic aliphatic phosphate coating produced by the method claimed in claim 4.

9. A concentrate for use in the make-up and replenishing of aqueous emulsions suitable for forming integral chemical coatings on metallic surfaces having lubricating properties which consists essentially of:

|                                  |        |     |    |
|----------------------------------|--------|-----|----|
| Lauryl acid phosphate            | grams  | 600 | 5  |
| Oleyl acid phosphate             | do     | 750 |    |
| Stearyl acid phosphate           | do     | 790 |    |
| Morpholine                       | do     | 150 |    |
| Sodium hydroxide                 | do     | 75  | 10 |
| Sodium acetate.3H <sub>2</sub> O | do     | 188 |    |
| Ferric nitrate.9H <sub>2</sub> O | do     | 188 |    |
| Distilled water                  | liters | 4   |    |

10. A concentrate for use in the make-up and replenishing of aqueous emulsions suitable for forming integral chemical coatings on metallic surfaces having lubricating properties which consists essentially of:

|                           |       |    |
|---------------------------|-------|----|
|                           | Grams |    |
| Monolauryl acid phosphate | 15    |    |
| Mono-oleyl acid phosphate | 7     | 20 |
| Morpholine                | 7     |    |

|                                  | Grams |
|----------------------------------|-------|
| Ferric nitrate.9H <sub>2</sub> O | 6     |
| NaOH                             | 1     |
| Distilled water to make 250 ml.  |       |

References Cited in the file of this patent

UNITED STATES PATENTS

|           |                 |               |
|-----------|-----------------|---------------|
| 1,900,973 | Bertsch         | Mar. 14, 1933 |
| 1,936,534 | Albrecht        | Nov. 21, 1933 |
| 2,080,299 | Benning et al.  | May 11, 1937  |
| 2,285,853 | Downing et al.  | June 9, 1942  |
| 2,328,540 | Hochwalt        | Sept. 7, 1943 |
| 2,432,784 | Miller et al.   | Dec. 16, 1947 |
| 2,452,321 | Kluge et al.    | Oct. 26, 1948 |
| 2,456,947 | Jernstedt       | Dec. 21, 1948 |
| 2,574,955 | Bishop          | Nov. 13, 1951 |
| 2,739,915 | Schuster et al. | Mar. 27, 1956 |

FOREIGN PATENTS

|         |               |               |
|---------|---------------|---------------|
| 732,286 | Great Britain | June 22, 1955 |
|---------|---------------|---------------|

UNITED STATES PATENT OFFICE  
CERTIFICATE OF CORRECTION

Patent No. 2,840,498

June 24, 1958

Earl Eugene Logue, Jr., et al

It is hereby certified that error appears in the printed specification of the above numbered patent requiring correction and that the said Letters Patent should read as corrected below.

Column 2, line 62, for "20" read -- 80 --; column 3, line 51, for "sever" read -- severe --; column 4, line 4, for "from" read -- form --.

Signed and sealed this 11th day of November 1958.

(SEAL)

Attest:

KARL H. AXLINE  
Attesting Officer

ROBERT C. WATSON  
Commissioner of Patents